

June 8, 1948.

J. P. CATLIN ET AL

2,442,841

METHOD OF NECKING AND TAPERING CARTRIDGE CASES

Filed Nov. 10, 1944



Fig. 1



Fig. 2



Fig. 4



Fig. 3



Fig. 4a

INVENTORS.  
JOHN P. CATLIN.  
GEORGE R. ECKSTEIN.  
MILTON B. VORDAHL.

*Harold J. Gamma*  
AGENT

## UNITED STATES PATENT OFFICE

2,442,841

METHOD OF NECKING AND TAPERING  
CARTRIDGE CASES

John P. Catlin, Fairfield, and George R. Eckstein,  
Bridgeport, Conn., and Milton B. Vordahl,  
Richland, Wash., assignors to Remington Arms  
Company, Inc., Bridgeport, Conn., a corpora-  
tion of Delaware

Application November 10, 1944, Serial No. 562,886

4 Claims. (Cl. 29—1.3)

1

The present invention relates, in general, to metal working and more especially to an improved method of making tubular metallic articles such as .50 caliber cartridge cases.

As an outgrowth of the scarcity of brass for the manufacture of cartridge cases, extensive work has been done to develop a satisfactory steel cartridge case. The use of steel has presented many problems not heretofore encountered in the manufacture of brass cases due primarily to the metallurgical characteristics of steel. It has been definitely established that a steel blank equal in diameter and thickness to a brass blank and subjected to cupping, drawing, annealing and tapering operations on the identical machines used in the manufacture of satisfactory brass cases behaves quite differently and regularly forms a case which is unsatisfactory both from the standpoint of ballistics and manufacture.

The manufacture of steel cartridge cases in quantity production lots and of a quality to meet Government specifications and to perform satisfactorily under the most severe tests has necessitated the development of new equipment and methods of manufacture.

The present invention relates particularly to an improved method of tapering and necking .50 caliber steel cartridge cases; however, it has been found that the method developed as hereinafter described is applicable and beneficial in the manufacture of cartridge cases of other materials such as brass and aluminum; and of other than standard specifications, cases of the latter type being termed cases of heavy geometry.

An object of the invention is the provision of an improved method of shaping metal tubular articles. A further object is to provide an improved method of tapering and necking steel cartridge cases.

Other objects, features and advantages of the invention will be described hereinafter in detail.

In the drawing:

Fig. 1 is a graph showing the body anneal and taper hardness pattern with conventional tapering.

Fig. 2 is a graph showing an unusually short zone of anneal and a taper hardness pattern with preworked tapering.

Fig. 3 shows a die stack for preworked tapering.

Fig. 4 shows schematically the four stages in tapering and necking a cartridge case in accordance with the method of this invention.

Fig. 4A is a schematic view showing the superposition of station 2 and station 4 of Fig. 4.

2

Briefly, cartridge cases are made by punching out a disk from a strip of metal and pressing the disk into the form of a cup. A preferred method and means of forming a cup from a steel blank for the manufacture of .50 caliber steel cases is described in detail in a copending application Serial No. 557,351, filed October 5, 1944, now Patent No. 2,415,940, issued February 18, 1947.

The cup is pressed or drawn through a plurality of dies until it becomes an elongated tube closed at one end. The closed end of the tube is bumped up to form the head of the case and suitable tapering and necking dies cold work the body of the case into its final shape. Metal becomes hardened when cold worked; moreover, to achieve the necessary hardness in the head and body of a steel case, the case, as drawn, that is to say after final draw, may be heated above the upper critical temperature and brine quenched. It has been the practice in making brass cartridge cases to anneal the case immediately preceding the tapering and necking operations. The purpose of such body anneal is two fold, first to facilitate the metal displacement necessary to tapering and necking, and second to prepare for the metallurgical properties required in different parts of the finished case. The head must be relatively hard for adequate strength, the body must approach the hardness of the head to secure the spring back which enables extraction and yet have sufficient elasticity for obturation, that is to say the ability to expand and form a gas seal between the outside 35 of the case and the wall of the chamber. The shoulder must be hard enough to give adequate longitudinal support against the impact of the firing pin, but neck and mouth must be soft enough to enable stretching to receive the bullet, crimping into the bullet, and expanding to release the bullet, all without rupture. And, finally, the body of the case must be of substantially uniform hardness to prevent longitudinal stretching and head set back on firing. These properties of a case are requisite for insuring good ballistic performance of the finished cartridge and a case having such properties is hereinafter referred to as a case having satisfactory ballistic performance.

Heretofore, the combination of an accurately controlled anneal pattern such as shown at A in Fig. 1 and the cold working done by the tapering and necking dies, as indicated at H, has produced brass cartridge cases free from cracks and having satisfactory ballistic properties. However, early

efforts to taper and neck a steel case by these accepted methods were unsatisfactory for, even with the most accurately controlled anneal pattern, steel cases were wont to evidence stretching, incipient wrinkling and excessive taper scrap.

The present invention relates primarily to the discovery that a cartridge case may be successfully tapered without requiring the critical anneal patterns heretofore considered indispensable to tapering operations, that is to say, the limitations which heretofore were required in an anneal pattern to insure successful tapering have been divorced from those limitations of the anneal pattern requisite for satisfactory ballistic performance.

As a result, a wider range of anneal patterns has been made available for obtaining improved ballistic properties in steel cartridge cases. As an example, Fig. 2 shows an anneal pattern providing an unusually short zone of anneal which is adapted to obviate longitudinal stretching by insuring uniform body hardness from head to shoulder.

It has been found that one way of successfully tapering and necking a case and in particular a steel case which has been quench hardened and stress relieved but not annealed; or which has been annealed primarily for ballistic performance is to subject the upper end only of the case to relatively severe or abrupt work hardening such that the yield stress of the metal is localized. As a consequence, a fold attempting to propagate itself in the body of the case during the tapering operation will run into relatively unstressed metal and be diffused as hereinafter described.

Referring to the drawings, Fig. 4 shows the four stages through which a .50 caliber steel case passes in being processed in accordance with the method of this invention from a substantially cylindrical quench hardened and stress relieved case shown at station 1 to the finished tapered and necked case shown at station 4.

The cylindrical case shown at station 1 is preferably annealed to build the desired ballistic qualities into the case and it is possible that the anneal pattern may be chosen so as to reduce the pressures on the tapering dies but, as indicated above, the discovery which characterizes the present invention is that the tapering of the case is practically independent of the conventional taper anneal and may be successfully accomplished without such anneal by subjecting the case to an abrupt work hardening in a limited region extending from the mouth of the case to a point *p* on the body which, as shown in Fig. 4, is somewhat lower than the shoulder *s* of the finished case. This abrupt work hardening is hereinafter termed "preworking" and is carried out by effecting an abrupt and relatively large reduction in diameter of a short portion *w* of the upper part of the case. In the embodiment shown in the drawings, this reduction in diameter is substantially 0.104 inch. One method of accomplishing this abrupt reduction in diameter is to suddenly impress a relatively severe taper on the upper end of the case. The taper shown and used to constrict the portion *w* of the case comprises an included angle of substantially  $14^{\circ} 30'$ . It will be understood, however, that the specific angle described is the preferred angle for successful operation of but does not constitute a limitation on the invention; and that other methods of abruptly work hardening the metal may suggest themselves as, for instance, by a sudden expansion of the metal.

The body of the case below the point *p* of the preworked region *w* has not been tapered or pre-

worked and hence is in its original hard, stress relieved and/or annealed condition. While the degree or severity of the preworking of the portion *w* of the case is greater than that done by the gradual tapering operations of conventional methods, nevertheless, the prework taper does not equal or exceed that of the final necking operation, as indicated in Fig. 4A lest otherwise the metal in the region corresponding to the shoulder *s* of the finished case be reduced or displaced so as to preclude the formation of a proper shoulder. It is well understood that the shape of the shoulder and the head to shoulder length is critical both from the standpoint of ballistics and successful operation in a firearm.

The preworking of the upper end of the case may be accomplished by means of a suitable die stack such as shown in Fig. 3 and which comprises a holder 10 having a top spacer block 11, a preworking die 12, a guide 13 and a bottom spacer block 14. The preworking die 12 comprises a tapered annulus having the aforesaid included angle of substantially  $14^{\circ} 30'$  and is adapted to be driven down over the mouth of a cylindrical case to abruptly form the relatively short steep taper *w*. The spacer blocks 11 and 14 in conjunction with suitable adjustments of the holder 10 in the reciprocating gate of the press (not shown) constitute means for holding the preworked taper *w* to a predetermined region on the upper end 15 of the case. The metal which is abruptly pre-worked by the action of the tapering die 12 is strained beyond the yield point elongation of the material which reduces the tendency of the metal to fold on subsequent tapering; and being confined to the upper end of the case localizes the yield stress set up in the case during tapering, that is to say, a stress set up in the preworked portion *w* of the case during the body tapering operation and tending to form incipient folds in 20 the metal will be dissipated as soon as it strikes 25 the unstressed body portion of the case.

The body tapering operation is carried out at station 3, see Fig. 4, at which a taper corresponding substantially to the taper put on the body 30 of a case at the last station in a conventional two stage tapering operation is impressed on the body 35 of the case, as shown at *b* in Figs. 4 and 4A.

Prior to the present invention, the body of a case has been tapered in two operations, namely 40 by an initial taper which partially tapers the body of the case and a final taper which completes the body taper and controls the head to shoulder length. In accordance with the method of this invention, the body of the case is tapered in a 45 single operation, the body taper formed at station 3 being the final taper put on the case. This has been made possible through the discovery that by preworking a limited portion of the neck of the case, the yield stress is localized, and hence 50 the propagation of taper folds in the body of the case during tapering is prevented. The taper operation also pulls in the preworked taper portion 55 *w* of the case so that it is substantially straight, as shown at station 3 in Fig. 4, the shoulder point 60 *p* being substantially eliminated.

The necking of the case and control of head to shoulder length is done at station 4, see Fig. 4, at which a necking die is brought down over the tapered case to reduce the neck *f* of the case to its final diameter and length and form the shoulder *s* at a predetermined distance from the head 65 of the case. This final operation corresponds in some respects to conventional methods by which cases are necked and the head to shoulder length controlled. It will be noted, however, that in as-

much as the body has been completely tapered at the preceding station, the necking operation and head to shoulder length control are done independently of the body tapering operation.

The method of tapering and necking cartridge cases and in particular .50 caliber steel cases by preworking enables the production of finished steel cases which are free from wrinkles or other visual defects and which have ballistic properties comparable to brass cases. Moreover, preworking has resulted in a remarkable reduction in taper scrap in the manufacture of steel cases and is applicable with equal success to brass or aluminum cases or cases of heavy geometry. And finally, preworked tapering enables steel cases to be tapered without being annealed thereby permitting a wider range of anneals from which to select patterns which will insure optimum ballistic performance.

The term "bottle neck cartridge case," used for simplicity in the appended claims, identifies a cartridge case as illustrated at stage 4 in Fig. 4; such case comprising a body or powder chamber of relatively large diameter joined by a tapering shoulder to a bullet receiving neck of relatively small diameter.

What is claimed is:

1. In the forming of a bottle neck cartridge case from a substantially cylindrical tubular blank, the method which comprises the sequence of steps of: subjecting the metal which subsequently forms the neck, shoulder and immediately adjacent portion of the body, to a severe cold working; tapering the entire body by a relatively slight cold working; and cold working the neck and shoulder to the desired finished dimensions.

2. In the forming of a bottle neck cartridge case from a substantially cylindrical tubular blank, the method which comprises the sequence of steps of: pre-stressing the neck and shoulder

forming metal beyond its yield point; tapering substantially the entire body; and forming the neck and shoulder to the desired finished dimensions.

5 3. In the forming of a bottle neck cartridge case from a substantially cylindrical tubular body of steel, the method which comprises the sequence of steps of: hardening by cold working the metal which subsequently forms the neck, shoulder and immediately adjacent portion of the body; tapering the entire body by a relatively slight cold working; and cold working the neck and shoulder to the desired finished dimensions.

10 4. In the forming of a bottle neck cartridge case from a substantially cylindrical tubular body of steel, the method which comprises the sequence of steps of: inducing by cold working a pattern of maximum stress in the neck forming portion, said stress diminishing through the shoulder forming portion and merging with unstressed metal in the portion of the body adjacent said shoulder; tapering the entire body by a relatively slight cold working; and cold working the neck and shoulder to the desired finished dimensions.

20 25 JOHN P. CATLIN.  
GEORGE R. ECKSTEIN.  
MILTON B. VORDAHL.

#### REFERENCES CITED

30 The following references are of record in the file of this patent:

#### UNITED STATES PATENTS

| Number       | Name      | Date          |
|--------------|-----------|---------------|
| 35 1,289,389 | Callerson | Dec. 31, 1918 |

#### OTHER REFERENCES

40 American Machinist, July 22, 1943, pp. 114-124,  
"Cartridge Cases for 37 mm. Shells." Published  
by McGraw-Hill, New York.